

June 2, 1953

W. O. BINDER

2,640,792

INERT MONATOMIC-GAS SHIELDED REFRACRY METAL  
REMELTING SURFACE-DEFECT REMOVAL PROCESS

Filed Jan. 29, 1951



INVENTOR  
WILLIAM O. BINDER  
BY  
*D. Harrison*  
ATTORNEY

## UNITED STATES PATENT OFFICE

2,640,792

INERT MONATOMIC-GAS SHIELDED REFRAC-  
TORY METAL REMELTING SUR-  
FACE-DEFECT REMOVAL PROCESS

William O. Binder, Niagara Falls, N. Y., assignor  
to Union Carbide and Carbon Corporation, a  
corporation of New York

Application January 29, 1951, Serial No. 208,395

1 Claim. (Cl. 148—10)

1

This invention relates to metal working, and more particularly to the removal of surface defects in refractory metal ingots by remelting the adjacent metal.

High-chromium alloys require careful surface conditioning prior to hot-rolling in order to ensure satisfactory surface quality. Because of their inherent resistance to oxidation, these alloys do not scale readily, hence they retain surface defects which normally are eliminated in the reheating furnaces in the case of more freely scaling metals. Most of the ingot defects causing surface rejections are laps and seams due to metal splashing. Since they are located near the surface, the standard commercial practice is to remove these defects mechanically by hand grinding with abrasive wheels. More recently, powder scarving techniques have been developed. However, both processes result in considerable loss of metal, and the hand-grinding process is slow, relatively costly, and presents labor problems due to the disagreeable nature of the work.

The corrosion resistance of stainless steels and related high-chromium alloys is a function of chromium content; higher chromium contents imparting greater resistance. Any impoverishment of the surface by oxidation of chromium would reduce the general corrosion resistance of the metal. In borderline cases, oxidation could reduce the concentration to a dangerous minimum. Loss of easily oxidizable metals such as columbium, titanium, and tantalum must also be avoided as their loss would have a dangerous effect on the corrosion resistance of the alloys.

High-chromium alloys always carry a certain percentage of carbon and nitrogen. These elements normally are kept in solid solution and do not seriously affect the corrosion resistance of the metal. On heating in certain temperature ranges, these elements combine with chromium and precipitate along the grain boundaries of the metal. The formation of carbides and nitrides depletes the areas adjacent to the grain boundaries of chromium. When exposed to certain media, these areas tend to dissolve leading to inter-granular corrosion of the metal. Commonly accepted means for preventing precipitation of chromium carbides and nitrides is to keep the percentages of carbon and nitrogen in the metal low. In some cases, columbium, tantalum, or titanium are added to combine with carbon and nitrogen as these elements form relatively insoluble carbides and nitrides. Any pickup of carbon or nitrogen in the melted surface would decrease the inter-granular corrosion resistance of the alloy. Such pickup cannot be avoided if a carbon arc is used.

It has also been proposed to remove such de-

2

fects from steel billets by melting the adjacent metal with an arc protected from the air by a stream of hydrogen. However, the latter is not suitable for high-alloy metals, due to contamination of the metal by such gas. Hydrogen, as well as nitrogen, pickup during melting is detrimental because they dissolve readily in molten high-chromium alloys and may produce porosity when the metal solidifies.

Excessive silicon pickup during melting must also be avoided, as it not only decreases general corrosion resistance in some media, but also it causes brittleness, decreases weldability and hot-workability. Silicon is apt to be picked up when slags are employed to protect the metal during melting.

High-chromium alloys are susceptible to cracking during hot-working if improperly melted and cast. Oxygen, carbon, and nitrogen have a direct influence, and the pickup of these elements should be kept to a minimum. Protective slags tend to oxidize the metal unless they are kept on the reducing side, and they do not prevent nitrogen pickup, particularly when the slag and metal are exposed to electric arc temperatures.

The main object of this invention is to provide an economical and efficient method of removing surface defects in high-alloy, refractory metal bodies by remelting the adjacent metal by means which yield the same composition in the melted as in the unmelted portions.

This is accomplished, according to the invention, by remelting the high-alloy metal in a shielding atmosphere consisting essentially of inert monatomic-gas of the class consisting of argon, helium, and mixtures thereof. While the metal can be melted by any suitable heating medium, the preferred expedient is an electric arc struck between a tungsten electrode and the metal body of sufficient current-carrying capacity to melt the metal in the area of the surface defect to be removed. Such arc and the molten metal are continuously shielded from the air by a stream of inert monatomic gas during such arc remelting operation. As a result, the defect is removed, leaving the metal that has been melted of the same composition as that of the base metal.

Summarizing, surface melting according to the invention in an inert monatomic gas atmosphere has the following distinct advantages: there is no loss of easily oxidizable metals, hence the metal retains its corrosion resistance; there is no porosity due to pickup of hydrogen or nitrogen; there is no pickup of carbon or nitrogen to cause inter-granular corrosion susceptibility; there is no loss of hot-workability due to oxidation of the metal; and since no slag is used, there is no problem due to entrapment of slag during solidification or to pickup of dele-

terious impurities present in the slag-making materials.

In the drawing, the single figure is diagrammatic view illustrating the invention.

As shown in the drawing, a metal body 10, such as billet is moved horizontally under a tungsten electrode 12 provided with a gas nozzle or cup 14. The body 10 and electrode 12 are connected by leads 16 and 18 to an electric power source 20 of sufficient current-supplying capacity to energize an electric metal melting-arc 22 between the surface of the body and the tip of the electrode during such movement of the work 10. Simultaneously therewith the arc and heated surface portions of the electrode and work are shielded from the air by an annular stream 24 of inert monatomic-gas which is delivered to the nozzle 14 from a suitable source via an inlet 26.

As the work 10 moves under the inert monatomic-gas shielded arc welding torch 28, the arc 22 melts the adjacent metal containing defects, forming a molten puddle 30 which progresses from one end to the other of the billet. Oxides and other foreign matter float out of such molten metal, leaving a "premelted," homogeneous surface 32 composed of metal of the same composition as that of the base metal, which may be a high-alloy metal, such as high-chromium alloy, by virtue of the inert-monatomic gas shield 24.

Hot-rolling tests on small ingots indicate that nickel rich iron-molybdenum, and related alloys can be satisfactorily surface-conditioned prior to rolling by remelting the surface of the ingot with a shielded arc, according to the invention, by using either argon or helium gas as the protective atmosphere. The surface can be pre-melted manually, but mechanized premelting is more satisfactory as it is subject to better control.

The amperage value of the current during remelting depends on the depth of penetration required to remove the surface defects. An arc current of 450 amperes using argon, and a  $\frac{3}{16}$ -in. diameter tungsten electrode will remove defects about  $\frac{1}{4}$  in. deep. Somewhat lower amperage may be used with helium for substantially the same depth of penetration.

The speed of melting depends on the surface condition of the ingot and the amperage of the arc current. A work-speed of 10 in./minute at 450 amperes has been found satisfactory for small ingots though somewhat faster speed can be employed with iron-molybdenum-nickel alloys. If the ingot surface is extremely poor, the speed of melting should be reduced below 10 in./minute to insure elimination of the deep-seated defects. High melting speeds tend to cause undercutting particularly in the case of nickel-rich alloys. The premelt beads should overlap to avoid crevices and cracking between beads.

Good shielding conditions must be maintained at all times. The distance between the gas outlet cone and ingot surface is critical and should be maintained as closely as possible, not exceeding  $\frac{3}{8}$  inch. Surfaces of satisfactory quality were obtained, according to the invention, with a gas flow of 25 cu. ft./hour with argon, and 40 cu. ft./hour with helium. No significant difference in the quality of the surface was noted between the ingots premelted in argon and in helium.

Precautions should be taken to minimize arc interruptions as the craters form areas of shallow surface cracking in the rolled surface.

However, the starting craters are relatively shallow and can be removed by grinding without too much difficulty prior to rolling, and in most instances, the craters formed at the end of each pass can be confined to the piped section which is eventually discarded. Another scheme is to tack-weld suitable metal pieces on the ends of the ingot for starting and stopping purposes.

In cases where the defects are relatively deep cracks, an electrode composed of metal of the same composition as that of the base metal can be used, without departing from the invention, to supply the additional metal required to fill such deep cracks. However, the electrode preferably is composed of tungsten containing significant amounts of oxidic materials, such as thoria, which improve arc stability and/or other additions which improve the operation of the electrode.

I claim:

Process of removing surface and subsurface defects including laps and seams due to metal splashing, from ingots composed of relatively high-alloy refractory metals prior to hot rolling in order to insure satisfactory surface quality of the resulting product without the loss of any of the refractory alloy metal thereof and without any change in the composition of the base metal, which comprises positioning the ingot so that the surface to be conditioned is uppermost and substantially level, striking a relatively heavy duty arc between such surface of the ingot and a refractory metal electrode composed of tungsten; continuously shielding such arc and the adjacent portions of the electrode and ingot with an annular stream of monatomic gas of the class consisting of argon and helium and mixtures of argon and helium discharged from a nozzle surrounding such electrode in spaced concentric relation therewith at a gas flow rate of twenty-five to forty cubic feet per hour, positioning the end of such nozzle as closely as possible to the surface of said ingot at a distance of not more than three-eighths of an inch, continuously moving said gas shielded arc with respect to the ingot surface at a speed of the order of about ten inches per minute while maintaining such critical spacing between said nozzle and the ingot surface, continuously supplying such arc with a current of the order of 400-450 amperes, deeply melting the ingot metal under such arc to a depth of the order of about one-fourth of an inch progressively and without interruption along the path of movement of such arc with respect to such surface, floating out oxides and other foreign matter, leaving a defect-free bead of homogeneous metal of exactly the same composition as that of the base metal and repeating such steps to form adjacent beads having laterally overlapping sides without crevices or cracks therebetween.

WILLIAM O. BINDER.

References Cited in the file of this patent

UNITED STATES PATENTS

| Number    | Name             | Date          |
|-----------|------------------|---------------|
| 1,512,787 | Morton           | Oct. 21, 1924 |
| 2,125,172 | Kinzel           | July 26, 1938 |
| 2,185,496 | Brown            | Jan. 2, 1940  |
| 2,405,542 | Wassell          | Aug. 6, 1946  |
| 2,474,023 | Wyer             | June 21, 1949 |
| 2,475,357 | Miller           | July 5, 1949  |
| 2,515,559 | Lancaster et al. | July 18, 1950 |
| 2,532,410 | Kennedy          | Dec. 5, 1950  |